

# UNITED STATES PATENT OFFICE.

LEOPOLD SCHMIED, OF PRAGUE, AUSTRIA-HUNGARY.

## PROCESS FOR THE MANUFACTURE OF BREWERS' PITCH.

No. 895,800.

Specification of Letters Patent. Patented Aug. 11, 1908.

Application filed June 7, 1907. Serial No. 377,803.

### BEST AVAILABLE COPY

*To all whom it may concern:*

Be it known that I, LEOPOLD SCHMIED, citizen of the Empire of Austria-Hungary, residing at Prague, Austria-Hungary, have invented 5 certain new and useful Improvements in the Process for the Manufacture of Brewers' Pitch, of which the following is a specification, reference being had therein to the accompanying drawing.

0 The present invention has for its object a process for the manufacture of brewers' pitch by the dry distillation of colophony, in which, as far as possible, all constituents of the colophony which are volatile at the 15 pitching temperatures are driven off while carefully maintaining low distillation temperatures, whereupon the distillation residue is mixed with paraffin in the well known manner.

20 In order to obtain brewers' pitch which is utilizable with the novel pitching methods in which temperatures exceeding 200° C. are employed, it is known to free resinous products from the constituents volatile at these 25 pitching temperatures by vigorous superheating. Owing to the great heat some carbonization, although only a little, takes place, which imparts a deep color to the residue. This is readily detected in all 30 superheated pitches on the market and in the mixtures made therefrom, as when dissolved these products leave a carbonaceous residue.

Hitherto it has been held that the constituents of resin which in applying pitch at high temperatures become volatile and which are consequently prejudicial for this purpose, were not distilled over until at a 35 temperature of 330° C. (temperature of the mass) and consequently that the carbonization which affects the flavor of the beer, was unavoidable; it was thought that it was 40 precisely high decomposition temperatures which were necessary for obtaining a residue 45 of good quality and that the pitch was favorably influenced by them. It has, however, been found that the constituents exerting an 50 unfavorable influence on the utilization as pitching medium distil over from colophony even at low temperatures if the distillation is carried out very slowly and so as to prolong its duration while carefully avoiding superheating, that is to say the temperature is not allowed to exceed 300° C. By this

means not only is any carbonization avoided, 55 but in addition the volatile constituents are driven off far more effectually than heretofore and the other properties of the product are also favorably influenced: for instance the residue in the still presents greater 60 tractability so that smaller quantities of paraffin need be added than to colophony or superheated pitches. The novel process is carried into practice by continuing the dry distillation of the colophony at temperatures 65 of 230°-300° C. until the loss of matter caused by the distillation amounts to 16-18%, while in the known process for manufacturing superheated pitch the loss by distillation may be taken as 11%. During this 70 operation a fraction of crude resin oil is distilled over in addition to the first running (acid water and pinolin). The residue in the still is then allowed to cool to 100°-120° C., whereupon it is melted with neutral paraffin 75 or a similar hydrocarbon until a homogeneous, varnish-like mass is formed.

The product by the above method shows a conchylaceous fracture and when dissolved does not leave a carbonaceous residue. Accordingly, contrary to what is the case with all superheated pitches hitherto known, which have a bitter taste caused by the carbonization, it does not impart any flavor to beer and wort even in a warm condition and 85 without previous swilling of the casks.

The coat of varnish produced by the application of the novel pitching medium is more 90 resistant and durable than the known coat of pitch, so that labor, time and material are 95 economized; but even for each pitching much less pitching medium is required than when superheated pitch is used. The coats are very thin and adhere well to iron and cement, so that the modern iron and cement 95 fermenting vats may be coated with the varnish.

Having now particularly described and ascertained the nature of my said invention and in what manner the same is to be performed, I declare that what I claim is:

The herein described process of producing an entirely neutral pitch which consists in subjecting colophony, consisting of the resin of the coniferæ which has been freed from acetic acid and turpentine oil by distillation, to dry distillation at a temperature not in excess of from 230 to 300° C. until all con-

stituents volatile at the pitching temperature have been driven off and the loss caused by distillation amounts to from 16 to 18 per cent, and melting the neutral tasteless residue which remains with a neutral paraffin-like hydro-carbon corresponding to the desired consistency of the pitch.

In testimony whereof I have hereunto affixed my signature in presence of two witnesses.

LEOPOLD SCHMIED.

Witnesses:

ADOLPH FISCHER,  
ARTHUR SCHWERZ.